

E. BERLINER.

JOINT.

APPLICATION FILED AUG. 11, 1908.

926,974.

Patented July 6, 1909.



Inventor

Emile Berliner

Witnesses

Albert Hopkins  
Mary W. Hammer

By Stewart & Mason

Attorneys

BEST AVAILABLE COPY

UNITED STATES PATENT OFFICE.

EMILE BERLINER, OF WASHINGTON, DISTRICT OF COLUMBIA.

JOINT.

No. 926,974.

Specification of Letters Patent.

Patented July 6, 1909.

Application filed August 11, 1908. Serial No. 447,950.

To all whom it may concern:

Be it known that I, EMILE BERLINER, a citizen of the United States, residing at Washington, in the District of Columbia, have invented certain new and useful Improvements in Joints, of which the following is a description, reference being had to the accompanying drawing and to the letters of reference marked thereon.

10 My invention relates to an improvement in joints for the parts of framing and especially for cross cylindrical braces.

My invention has been especially designed for use in connection with flying machines. 15 The framework of such machines must of necessity, be very light, but of great strength. The material best adapted therefor for strength and lightness, is bamboo, which comes in long cylindrical strips. By reason 20 of their shape, it is very difficult to rigidly secure these strips together at the places where they must cross and the object of my invention is to provide a means for securing such pieces together at their crossing, al- 25 though it will be understood that the invention is applicable to other material than bamboo.

The invention therefore, consists in the matters hereinafter described and referred 30 to in the appended claims.

The invention is illustrated in the accompanying drawings in which;

Figure 1 is a side view illustrating the first step in the operation of forming the joint. 35 Fig. 2 is a similar view illustrating the second step; and Fig. 3 is a view illustrating the third step.

In these drawings, A represents two bamboo strips which are to be united at their 40 point of crossing. I first pass through the tubes at their point of crossing, a bolt *a* or nail or screw to temporarily hold them in proper position, although it will be understood that said step is not absolutely essential. 45 I then apply in a semi plastic condition around the joint in sufficient quantity, a mixture of shellac or other resinous substance, with a filler of oxid of iron or another oxid such as barium oxid or baryta,

sulfate of lead or zinc, or similar mineral substances, and a fibrous material, such as wool or cotton flock. The shellac or other resinous substance, acts as a binder, the mineral substance as a filler, and the wool or cotton flock, as a fibrous strengthener. 55 The mixture is formed in substantially the proportion of 5½, 10 and 1, respectively, of resinous substance, filler and fibrous substance by weight. Such a mixture is soft when heated and very tough and hard when cold. A wad of this mixture is softened by heat and placed around the joint as shown in *b* and pressed into place filling all the interstices in the material. Before it is cool and therefore hard, tape or cord or other 60 suitable binding material, as shown at *c*, is tightly wound around it and the bamboo, to press and hold the substance in place, and when cooled, the mixture becomes very hard, and an absolutely secure and rigid 70 joint is formed.

While I have described the use of the tape or cord, it will be understood that this may be dispensed with, although it aids in forcing the semi-plastic mass into the interstices of the wood, and also acts as a cover to prevent breaking of the mixture, which becomes somewhat brittle, when cool.

Having thus particularly described my invention, what I claim as new and desire to 80 secure by Letters Patent is:

1. A joint for cross bars, including a securing material of a resinous compound pressed around the joint.

2. A joint for cross bars including a securing material, consisting of a resinous substance and a fibrous substance pressed around the joint.

3. A joint for cross bars including a securing material consisting of a resinous substance and a mineral substance pressed around the joint.

4. A joint for cross bars, including a securing material composed of a resinous compound containing a filler, and a fiber pressed around the joint and a binding cord or tape encircling the same.

5. A joint comprising the cross bars, a se-

curing mixture surrounding the same, composed of shellac, oxid of iron, and flock pressed into shape around the joint.

6. The process of uniting cross bars, consisting in first holding them in position, then surrounding the joint with a warm semi-plastic mixture of suitable material, substantially as described, which becomes hard

when cool, and finally binding the joint with tape or the like.

In testimony whereof I affix my signature, in presence of two witnesses.

EMILE BERLINER.

Witnesses:

A. M. PARKINS,  
C. L. STURTEVANT.